

## UNITED STATES PATENT OFFICE.

GEORGE I. RAY, OF CHARLOTTE, NORTH CAROLINA, ASSIGNOR TO RADIATOR SPECIALTY COMPANY, OF CHARLOTTE, NORTH CAROLINA, A CORPORATION OF NORTH CAROLINA.

## COMPOSITION FOR REPAIRING LEAKS.

No Drawing.

Application filed April 12, 1927. Serial No. 183,243.

This invention relates to composition for stopping leaks in hot water circulating systems, especially for automobile radiators, engine blocks for internal combustion engines, 5 hot water heating systems, pumps, and in fact in every system in which the circulating medium is hot water.

An object of my invention is to provide a leak stopping composition which will work 10 well under all conditions, and one which will not clog or gum the system, as has been the case in many of the leak stopping compositions which have heretofore been on the market.

15 It is another object of this invention to provide a leak stopping composition for hot water circulating systems which will not only repair all leaks which may be present in the system at the time this composition is placed therein, but which will prevent leaks from forming while this composition is in the system, and which will also keep the interior of the system cleansed and in good condition.

20 I attain the above stated objects by mixing a composition of aluminum, flax seed meal, trisodium phosphate, soda ash and soap and placing the same in the hot water circulating system. The above ingredients will produce 25 the desired effects when the proportions are varied greatly, but I find that the most desirable proportions are as follows:

|                      | per cent. |
|----------------------|-----------|
| Aluminum             | 12        |
| Flax seed meal       | 50        |
| Tri-sodium phosphate | 15        |
| Soda ash             | 12        |
| Soap                 | 11        |

40 When this composition is placed in a hot water circulating system containing a quantity of water, the last three named ingredients dissolve and form a colloidal solution. The soap, stimulated and strengthened in its 45 action by the tri-sodium phosphate and the soda ash, exerts a strong suspending and cleansing action. The suspending action prevents the agglomeration of the insoluble materials in the mixture, and therefore, prevents the stoppage of the circulatory system. The insoluble materials are left as a somewhat fluffy mixture and are stirred up by the circulation of the system. The suspended 50 particles work their way into the leaks in the

system and there become lodged, the smaller 55 particles following the larger ones until the leak is entirely stopped.

The alkaline solution, caused by the presence of the tri-sodium phosphate and the soda ash, will slowly attack the aluminum particles in the sealed leaks, the carbonate forming the aluminum hydroxide and insoluble aluminum soap, and the presence of the phosphate resulting in the formation of aluminum phosphate. These agents, working together, 60 65 make a very permanent seal for the leaks.

The moderately alkaline solution prevents any separation of the fatty acids of the soap and helps to prevent the formation of any oily or greasy deposit on the inner walls of 70 the hot water circulating system. The phosphate, the carbonate and the soap produce a very efficient suspending agent for the insoluble matter, and also have a very satisfactory cleansing action on the interior of the 75 hot water circulating system.

If the soda ash were omitted from the mixture the solution would not be quite as alkaline, and the action of the aluminum would be somewhat lessened, which would be quite desirable in aluminum head engines. Also the sealing of the leaks would be accomplished more by the aluminum phosphate and less by the other compounds if the soda 80 ash were omitted.

85 In the specification I have set forth a preferred embodiment of my invention, and although specific terms are employed, they are used in a generic and descriptive sense, and not for purposes of limitation, the scope of 90 the invention being set forth in the appended claims.

I claim:

1. A composition for stopping leaks in hot water circulating systems comprising a mixture of aluminum, flax seed meal, tri-sodium phosphate, soda ash and soap. 95

2. A composition for stopping leaks in hot water circulating systems comprising a mixture of aluminum, flax seed meal, tri-sodium phosphate and soap. 100

3. A composition for stopping leaks in hot water circulating systems comprising a mixture of aluminum, flax seed, soda ash and tri-sodium phosphate. 105

In testimony whereof I affix my signature.

GEORGE I. RAY.